

# United States Patent Office

3,379,518

Patented Apr. 23, 1968

1

3,379,518

## ALUMINUM ALLOY

Frederick John Kranich, Chicago, Ill., assignor to Alum-alloy Company, Chicago, Ill., a partnership  
No Drawing. Filed Mar. 8, 1966, Ser. No. 532,596  
4 Claims. (Cl. 75—142)

This invention relates to aluminum alloys and concerns a particular aluminum alloy suitable for foundry work and having several long-sought advantages heretofore unavailable in a light-metal casting material.

The main objects of this invention is to provide an improved aluminum alloy capable of better sand and permanent mold castings for the foundry industry, which castings will be dimensionally stable after a short period of natural aging and will have a relatively high density.

It is another object of this invention to provide an aluminum casting alloy which has a high wear resistance under severe conditions of abrasion and also has high resistance to both acid and alkali corrosion; and to provide such an aluminum alloy that is free machining and which will not distort under cold or heat.

In the attainment of an aluminum alloy having these characteristics I have found a combination of elemental constituents that appears to be critical in so far as identity is concerned if the maximum advantage of each desired characteristic is to be had. I have also found that the basic material must be substantially pure virgin aluminum, 99.6% pure, and that the proportions of alloying ingredients for a melt of any size must be carefully maintained for the best practical results. Commercial aluminum should not be used since its inherent impurities will cause a loss of much of the before-mentioned desired characteristics.

According to my invention, for casting purposes, my improved aluminum alloy consists of the following materials, within the ranges stated, for a batch or melt of predetermined size:

|           | Percent by weight |
|-----------|-------------------|
| Beryllium | 0.05—0.08         |
| Copper    | 1.60—1.68         |
| Silicon   | 0.10—0.18         |
| Nickel    | 0.42—0.48         |
| Silver    | 0.20—0.30         |
| Magnesium | 1.10—1.18         |
| Titanium  | 0.15—0.19         |
| Aluminum  | Balance           |

The ranges stated for these ingredients of my improved aluminum alloy appear to be critical for maximum results and it should be noted that in any case 99.6% pure virgin aluminum should be used. Old aluminum or the usual commercial grades will produce inferior castings which lose many of the desired characteristics of the alloy produced according to my invention because of the impurities which aluminum contain. Also, I have found that too much copper will so reduce the capillary action as to make the metal sluggish in the mold; and that too much silicon will make the castings too brittle for uses where wear and corrosion resistance is most desirable. I have found too that a greater quantity of magnesium than that specified above will result in a proportionate decrease of corrosion resistance under both acid and alkaline conditions. The stated proportions of silver and nickel have been found to be just enough to produce good solid castings of optimum quality and a greater quantity of these materials than that specified would merely be a waste.

An optimum formula for my improved alloy is as fol-

2

lows, the proportions being in percentages of the total melt:

|           | Percent |
|-----------|---------|
| Beryllium | 0.06    |
| 5 Copper  | 1.65    |
| Silicon   | 0.12    |
| Nickel    | 0.44    |
| Silver    | 0.25    |
| Magnesium | 1.11    |
| Titanium  | 0.16    |
| Aluminum  | Balance |

When making the improved alloy the pure aluminum should be melted down to a liquid state at a temperature of about 1450° F. This heat should never exceed 1530° F. so that oxidation of the aluminum will be minimized. The presence of the oxide will show on the surface of the casting and also is detrimental to tensile strength. When the aluminum is melted the alloying materials are then added, and when the entire batch is molten it is ready to be poured in a normal casting procedure.

A typical melt of small size may be made as follows:

To 80 pounds of pure virgin aluminum, melted down to liquid state at 1450° F. add 16 ounces of beryllium copper containing 2 1/4% beryllium, 8 ounces of silicon copper containing 25% silicon, 10 ounces of titanium aluminum containing 25% titanium, 30 ounces of nickel aluminum containing 25% nickel, 4 ounces of silver, and 15 ounces of magnesium.

From the foregoing it will be seen that the source of beryllium and silicon is also the source of the copper for the improved alloy. The titanium aluminum compound is used as a titanium source to obviate the entry of iron into the alloy; and the nickel aluminum compound is used because of its lower melting point than that of pure nickel. The size of the melt may be varied to substantially any desired extent by merely varying proportionately the above stated quantities of the several ingredients.

Castings made from this alloy, when allowed to naturally age for a period of ten to twenty days, according to the weight and size of the cast product, are found to have all of the desired characteristics which were the objectives sought in the course of my development of the present invention, including complete stability against dimensional change. Additionally these castings exhibit a very high salt resistance and a remarkably high resistance to abrasion and wear. Other physical properties of my new aluminum alloy are as follows:

|                                                                 |         |           |
|-----------------------------------------------------------------|---------|-----------|
| Tensile strength (minimum)                                      | p.s.i.  | 28,433    |
| Corrosion test at pH 7                                          | hours   | 72        |
| Density                                                         | gm./cc. | 2.73      |
| Hardness (500 kg. load)                                         | B.H.N.  | 69        |
| Pouring temperature (preferred pouring temp. is about 1260° F.) | ° F.    | 1250—1350 |
| Solidification range of density                                 | ° F.    | 1160—1015 |

My improved aluminum alloy is particularly useful for pistons and pump impellers, particularly for impellers of pumps in sewage disposal plants, steel mills, and similar places where the pumpage is high abrasive or highly acid. For such uses impellers of my improved alloy have outlasted impellers made of manganese steel, and operating under identical conditions, by more than four times the life of the latter material. Other uses for which my improved alloy has been found to be exceptionally well suited as in various marine applications where high resistance to salt water corrosion is a necessity. My new aluminum alloy has the additional advantages of excellent machineability and good impact strength as well as the fact that it has and retains a bright white color.

Having thus described my invention what is claimed

as new and desired to be secured by Letters Patent is defined as follows:

I claim:

1. An alloy consisting of about 0.05% to about 0.08% by weight beryllium, about 1.60% to about 1.68% by weight copper, about 0.10% to about 0.18% by weight silicon, about 0.42% to about 0.48% by weight nickel, about 0.20% to about 0.30% by weight silver, about 1.10% to about 1.18% by weight magnesium, about 0.15% to about 0.19% by weight titanium, and the balance being aluminum.

2. An aluminum alloy according to claim 1 consisting of the following materials:

|                   | Percent by weight |
|-------------------|-------------------|
| Beryllium         | 0.05-0.08         |
| Copper            | 1.60-1.68         |
| Silicon           | 0.10-0.18         |
| Nickel            | 0.42-0.48         |
| Silver            | 0.20-0.30         |
| Magnesium         | 1.10-1.18         |
| Titanium          | 0.15-0.19         |
| Aluminum (virgin) | Balance           |

3. An alloy according to claim 1 wherein the components are in the following proportions by weight: 0.06% beryllium, 1.65% copper, 0.12% silicon, 0.44% nickel, 0.25% silver, 1.11% magnesium, 0.16% titanium, and the balance is substantially pure aluminum.

4. An alloy according to claim 1 wherein the ingredients are in the following proportions: beryllium, 0.06%; copper, 1.65%; silicon, 0.12%; nickel, from about 0.42% to 0.48%; silver from about 0.20% to about 0.30%; magnesium, 1.11%; titanium, 0.16%; and the balance is substantially pure aluminum.

#### References Cited

##### UNITED STATES PATENTS

|    |           |         |                 |        |
|----|-----------|---------|-----------------|--------|
| 15 | 2,383,026 | 8/1945  | Toleik          | 75-142 |
|    | 2,522,575 | 9/1950  | Hall et al.     | 75-142 |
|    | 3,172,790 | 3/1965  | Gilmore et al.  | 75-142 |
|    | 3,288,601 | 11/1966 | Flemings et al. | 75-142 |

20 HYLAND BIZOT, *Primary Examiner.*

RICHARD O. DEAN, *Examiner.*